

## UNITED STATES PATENT OFFICE

2,606,854

## COLORATION OF SHEET MATERIALS

John Allan, Spondon, near Derby, and Horace Finningley Oxley, Charmouth, England, assignors to Celanese Corporation of America, a corporation of Delaware

No Drawing. Application April 29, 1949, Serial No. 90,534. In Great Britain May 10, 1948

2 Claims. (Cl. 154—99)

1

This invention relates to the colouration of transparent or translucent sheets of thermoplastic derivatives or like polymers.

The various methods hitherto available for locally colouring sheet materials of the kind referred to above, and especially the methods available for printing rigid sheets have been defective with respect to the bloom, transparency and fastness to rubbing of the colourations obtained.

We have found that local colourations of very good bloom, transparency and fastness to rubbing can be obtained on such materials by transferring to selected areas of the sheet, a dye soluble in the sheet-material unaccompanied by any substance insoluble in said material, and simultaneously or subsequently subjecting the sheet to pressure applied by means of a polished surface at a temperature above the flow-point of the sheet material. By the flow-point of the sheet material is meant the temperature at which that material will flow 1" in a  $\frac{1}{8}$ " diameter tube in 2 minutes under a pressure of 1000 lbs. per square inch.

The invention will be described with particular reference to colouring sheets of plasticised cellulose acetate.

One method of carrying out the invention is to press on to the sheet material a cellulose acetate fabric printed with colours soluble in cellulose acetate, the pressure and temperature being sufficient to cause the plasticised cellulose acetate to flow without melting the cellulose acetate fabric. Thus, for example, a cellulose acetate fabric printed with the desired pattern in water-insoluble dyes having affinity for cellulose acetate, steamed, washed and dried, may be laid upon the sheet of cellulose acetate to be printed and the assembly placed between highly polished steel platens in a steam-heated press and pressed at 150 to 180° C. under 150 to 300 lb. per square inch pressure for a few minutes. After removing the assembly from the press and allowing it to cool, the fabric can readily be separated from the sheet material which will be found to have taken the design of the printed fabric in bright transparent colour, and to show also an attractive embossed fabric-effect.

The preliminary printing of the cellulose acetate fabric may be carried out in the ordinary way using a printing paste thickened, for example, with methyl cellulose or other suitable thickener. If attempts are made to print directly on to cellulose acetate sheet using pastes containing such thickeners, i.e. thickeners which are incompatible with the sheet-material, the

2

presence of the thickener on the printed sheet mars the effect obtained, giving an undesirable dullness to the colourations. When however, the design is transferred from a printed fabric as described, this dulling of the colours does not occur.

If, instead of using a fabric of cellulose acetate a printed cotton fabric is used, difficulty is experienced in separating the fabric from the printed sheet material. This difficulty can be somewhat reduced by using a fabric of tight-twisted Egyptian yarns well singed. The same difficulty is experienced when the printed fabric is replaced by a printed paper. In this case it is of some advantage to use a heavily pigmented paper heavily calendered, but neither with an Egyptian cotton fabric of the kind specified nor with a pigmented paper print have the results been nearly as satisfactory as when a printed cellulose acetate fabric is used. Linear polymers in which the dyes used are soluble, e.g. nylon, can be used successfully. Other linear polymers having the desired solubility properties include: other lower fatty-acid esters of cellulose i.e. esters derived from fatty-acids containing 2 to 4 carbon atoms, e.g. cellulose propionate, cellulose butyrate, cellulose acetate-propionate or cellulose acetate-butyrate, as well as cellulose ethers such as ethyl cellulose and benzyl cellulose.

30 A second method of carrying out the invention is to print the required design on a polished metal plate, e.g. by screen printing, in the form of a cellulose acetate lacquer, or other lacquer, which is compatible with the material of which the sheet is composed (by which is meant that all the constituents of the lacquer are soluble in the sheet-material), and after drying, to assemble the plate in contact with the sheet to be coloured in a heated platen press and subject the assembly to heat and pressure as described above. On removing the assembly from the press, cooling and separating the metal plate from the cellulose acetate sheet, the sheet is found to exhibit the desired colour effects.

45 A further method of carrying out the invention is to print directly on to the cellulose acetate sheet by the silk-screen process using a cellulose acetate lacquer compatible with cellulose acetate and containing a dye which is soluble in cellulose 50 acetate, and after the print has dried, to press the printed sheet between polished metal platens at such temperatures and pressures as are referred to above. In this way also colour effects are obtained which are bright, transparent, and 55 remain fast to rubbing. This method can be ap-

plied to unpolished sheets as obtained from a block-slicing operation to give printed sheets of very satisfactory finish.

An essential feature of the invention is the use as the colouring agent of a dye which is soluble in the sheet-material to be coloured. For cellulose esters and ethers those azo-dyes, nitro-diarylamine dyes, and amino-anthraquinone dyes, which are water-insoluble and have affinity for the cellulose derivative, are generally suitable, and many of these dyes are also suitable in the colouration of sheets having a basis of a condensation polymer such as nylon or an addition polymer such as polymethyl methacrylate.

Although the transfer with the colour of any substance incompatible with the cellulose derivative or other polymer is to be avoided if colourations of high transparency are required, the invention includes a process in which a pigment, especially a white pigment is transferred to the sheet material in areas along-side the areas coloured by the dye. The most attractive effects have been obtained using pigments of high refractive index, e. g. titanium dioxide of refractive index greater than 2. The pigment may, for example, be contained in a lacquer used to print directly onto the cellulose acetate sheet or may be used in preparing a printing plate for printing a coloured design upon the sheet material.

The following examples, in which all the parts are by weight, illustrate the invention:

#### Example 1

A plain woven cellulose acetate fabric was printed with a paste of the following composition:

200 parts 4-nitro-2'-chlor-4'-dioxy ethylamino-  
azo-benzene  
80 parts water  
120 parts ethyl alcohol  
24 parts methyl cellulose

The printed fabric was then steamed to fix the colour, washed and dried.

On the lower platen of a steam heated press were assembled in the following order:

3 sheets of cellulose pulp;  
A polished stainless steel platen;  
The printed fabric with the printed face upper-  
most;  
A sheet of plasticised cellulose acetate 4 mm.  
thick.

The press was then closed and the assembly subjected to a pressure of 200 lb. per square inch for two minutes at 180° C. The press was then opened, the assembly allowed to cool and the fabric separated from the sheet.

In this way a coloured pattern of fine bloom and transparency was obtained on the cellulose acetate sheet. The sheet showed also an attractive embossed effect derived from the structure of the fabric.

The cellulose acetate fabric can be replaced by a fabric of poly-hexamethylene adipamide.

#### Example 2

The process was carried out as in Example 1, except that the cellulose acetate fabric was printed also in areas along-side the coloured areas with a paste of the following composition:

200 parts of a 50% aqueous titanium dioxide paste  
80 parts of a 60% aqueous albumin paste  
8 parts ammonium hydroxide

30 parts glycerol  
82 parts water  
24 parts methyl cellulose

During the pressing operation the titanium dioxide was transferred to the cellulose acetate sheet forming areas of dull lustre alongside the areas of bright transparent colour.

#### Example 3

A pattern was formed by screen printing on to a metal printing plate the following composition:

60 parts 4-nitro-2'-chlor-4'-dioxy ethylamino-  
azo-benzene  
60 parts cellulose acetate  
16 parts dimethyl phthalate  
4 parts triphenyl phosphate  
270 parts acetone  
280 parts ethyl lactate  
20 parts glycol diacetate

A sheet of plasticised cellulose acetate of a thickness of 4 mm. was laid on a polished stainless steel platen; the screen-printed metal plate was placed with the printed surface downwards on the cellulose acetate sheet, and the assembly was pressed in a steam-heated press at a temperature of 180° C. under a pressure of 200 lb. per square inch for two minutes.

The press was then opened, the assembly allowed to cool and the cellulose acetate sheet removed. In this way, bright colourations similar to those of Example 1 were obtained.

#### Example 4

A rigid unpolished sheet of plasticised cellulose acetate, sliced from a block, was screen printed with the composition of Example 3. The printed sheet was allowed to dry and was then inserted between two polished stainless steel platens in a steam-heated press. The sheet was pressed at about 180° C. under a pressure of 200 lbs. per square inch for two minutes.

In this way the sheet was given a high polish on both surfaces and a coloured pattern of high transparency and bloom on one surface.

#### Example 5

The process was carried out as in Example 4, save that the lower platen, instead of being polished, was engraved with a fine pattern so as to roughen the whole lower surface of the cellulose acetate sheet. The effect was to increase the brightness of the colourations when viewed by reflected light.

#### Example 6

The process was carried out as in Example 3, except that, after printing the plate with the coloured composition, it was also screen-printed with the following composition:

60 parts milled titanium dioxide  
60 parts cellulose acetate  
16 parts dimethyl phthalate  
4 parts triphenyl phosphate  
280 parts ethyl lactate  
240 parts acetone  
20 parts glycol diacetate

Using this printing plate, colourations similar to those referred to in Example 3 were obtained with areas of low lustre alongside the coloured areas.

#### Example 7

The process was carried out as in Example 5, except that after printing with the coloured com-

position, areas alongside the coloured areas were printed with the titanium dioxide composition of Example 6. A highly polished sheet with a pattern comprising brightly coloured areas and areas of dull lustre was obtained.

In these examples the cellulose acetate sheet material can be replaced by sheet material having a basis of cellulose acetate-butyrate, cellulose acetate-propionate, cellulose propionate or polymethyl methacrylate, and the dye specified can be replaced by 2:4-dinitro-4'-amino-diphenylamine, 1:4 - dimethylamino - anthraquinone or alpha-1-ethylaminoanthraquinone. Any of the cellulose esters specified can be used as the basis of the lacquers used in Examples 3 to 7 instead of cellulose acetate.

The brightness of the colourations obtained when viewed by reflected light may be increased by roughening the uncoloured surface of the sheet. This may be done, for instance, as illustrated in Example 5, by pressing that surface against a hot surface having the necessary rough texture.

The process of the invention may be employed in the colouration of thick, substantially rigid transparent or translucent thermoplastic sheet material as well as of thin, flexible films (including foils).

Having described our invention, what we desire to secure by Letters Patent is:

1. Process for locally colouring self-supporting sheets of a plasticized cellulose fatty-acid ester in which the acid radical contains 2 to 4 carbon atoms, which comprises printing onto a textile fabric of cellulose acetate a counterpart of the

coloured pattern required, putting together the coloured surface of the fabric and that surface of the sheet which is to be coloured, applying pressure to the back surface of the fabric by means of a polished surface at a temperature above the flow-point of the sheet-material to cause transfer of the dye from the fabric to the sheet, and separating the fabric and sheet.

2. Process according to claim 1, wherein the fabric before being brought into contact with the sheet is printed also with a white pigment of refractive index at least 2, in areas alongside the coloured areas and said pigment is transferred from the fabric to the sheet during the pressing operation.

JOHN ALLAN.

HORACE FINNINGLEY OXLEY.

#### REFERENCES CITED

20 The following references are of record in the file of this patent:

#### UNITED STATES PATENTS

| Number    | Name           | Date          |
|-----------|----------------|---------------|
| 1,883,854 | Michael        | Oct. 18, 1932 |
| 1,981,472 | Schneider      | Nov. 20, 1934 |
| 2,353,717 | Francis et al. | July 18, 1944 |
| 2,404,073 | Karfiol et al. | July 16, 1946 |
| 2,510,750 | Marquardt      | June 6, 1950  |

#### FOREIGN PATENTS

| Number  | Country       | Date         |
|---------|---------------|--------------|
| 562,573 | Great Britain | July 6, 1944 |